

Sept. 27, 1932.

J. E. GROSS

1,879,740

LUMINOUS TUBE

Filed Nov. 2, 1928

Fig. 1.



Fig. 2



Fig. 3.



Fig. 4.



INVENTOR

Joseph E. Gross.  
BY Birney Hines

ATTORNEY

## UNITED STATES PATENT OFFICE

JOSEPH E. GROSS, OF SWISSVALE, PENNSYLVANIA, ASSIGNOR TO AURORA SIGN COMPANY, A CORPORATION OF PENNSYLVANIA

## LUMINOUS TUBE

Application filed November 2, 1928. Serial No. 316,707.

My invention relates to electrically operated gas-filled luminous tubes and more particularly to electrodes for such tubes.

It is the object of my invention, in general, to provide a luminous tube that shall be simple and efficient in operation and capable of being readily and economically manufactured and maintained.

A more specific object of my invention is to provide a luminous tube in which a minimum amount of sputtering will occur during its operation.

Another object of my invention is to provide a luminous tube in which the disintegration of the electrodes shall be practically negligible.

It is also an object of my invention to provide a luminous tube that may be operated by a minimum amount of auxiliary apparatus.

Other objects of the invention will, in part, be obvious, and will, in part, appear hereinafter.

For an illustration of one of the various forms my invention may take, reference may be had to the accompanying drawing, in which;

Figure 1 is a top plan view, partially broken away, of a luminous tube embodying my invention;

Fig. 2 is a view taken along the line II—II of Fig. 1;

Fig. 3 is a view taken along the line III—III of Fig. 1; and

Fig. 4 is a view taken along the line IV—IV of Fig. 1.

In the drawing, I have illustrated a luminous tube as comprising an elongated sealed glass envelope 1 that is adapted to be exhausted of air and gases to a predetermined value and then filled with a predetermined amount of a monatomic gas such as neon, argon or helium.

The glass envelope 1 is provided with enlarged end portions 2 and 3 in which are disposed, respectively, a cathode 4 and an anode

5, both of these electrodes being connected to the secondary circuit of a transformer 6 by a pair of lead-in wires 7 and 8.

As shown, the cathode 4 is disposed in an elongated cavity 9 in a supporting member 10 of a suitable insulating material, such as porcelain. The porcelain member 10 is mounted on and fused to a glass press 11 that constitutes a part of the glass envelope 1. A conductor 12 that is disposed in a longitudinal aperture in the supporting member 10 serves to connect the cathode 4 to the lead-in wire 7.

It will be noted that the cavity 9 is of such shape and dimensions that the member 10 covers the cathode 4 to such an extent that only a small area of its total surface is exposed and therefore that the member 10 not only acts as a support for the cathode but also serves as an insulating cover or casing to limit or restrict the surface of the cathode that is exposed to the gas with which the lamp may be filled. This provision for covering the cathode by an insulating material to such an extent that only a small portion of its entire surface is exposed is important, in that it limits the area of the cathode from which the electrical discharge may pass when the tube is placed in operation, and therefore conserves the heat in the cathode to such a degree while the tube is being started that it is not necessary to employ a heater for the cathode or a large kindling current. I have found that the exposed area of the electrode should be at least less than one square decimeter per ampere.

I have also found that especially efficient operation of the tube may be obtained by placing the cathode 4 so far within the cavity 9 that the material surrounding the mouth of the cavity provides a restricted passage-way for the discharge from the exposed surface of the cathode.

In constructing the cathode 4, I prepare a mixture of a suitable metal, such as nickel,

and suitable salts, such as barium carbonate and strontium carbonate. While the materials referred to may be employed in various combinations, I prefer to employ a mixture of approximately the following proportions, by weight, nickel 50 percent, barium carbonate 25 percent and strontium carbonate 25 percent. The ingredients are mixed together thoroughly and then tamped into the cavity 9 in the porcelain member 10 until the cavity is filled to within a short distance of its mouth, so that the porcelain around the mouth of the cavity will extend a sufficient distance to constitute a tube or restricted passageway through which any discharge from the cathode must pass.

After the mixture is tamped down in the cavity 9 of the member 10, it is strongly heated until it becomes a sintered mass of nickel, barium oxide, and strontium oxide. Upon completion of the sintering process, the supporting member 10 carrying the cathode 4 and the press 11, upon which it is mounted, are placed in position in the tube and the press 23 is fused to the glass envelope 1.

Any suitable electrode may be employed as the anode 5 in the tube, but I prefer to use an anode constructed in the same manner as the cathode just described, as it simplifies 30 the manufacturing activities necessary to produce a satisfactorily operative tube.

After the anode and the cathode are placed in position in the glass envelope, the tube may be exhausted, filled with gas and sealed off in the usual manner.

Upon operatively connecting the completed tube to a suitable source of electrical energy, such as the transformer 6, the voltage rises rapidly for a small fraction of a second until 40 the breakdown of the gap between the electrodes occurs. After the breakdown occurs, the voltage drops to a value determined by the size of the tube and the electrodes. Inasmuch as the exposed surface of the cathode 4 is very limited, the discharge is restricted to such a small area that it heats rapidly to such a degree as effects a discharge of electrons from that surface and thereby causes the gas in the tube to become luminous.

50 By reason of the small exposed area of the cathode and the short period during which the voltage rises, such disintegration of the cathode as occurs in operating the lamp is practically negligible and the life of the tube will not be shortened by an excessive deposit on its interior surface.

As shown, however, the body of the cathode 4 extends within the cavity 9 for such a distance as will insure a supply of active material during the full life of the tube regardless of any disintegration of the small exposed discharge area of the cathode that may take place.

It will therefore be seen that I have provided a luminous tube that is easily manufac-

tured, that is simple in operation and which will have exceptionally long life.

While I have illustrated and described only one specific embodiment of my invention, I realize that it is susceptible of wide application, and I do not desire to be limited to the precise construction illustrated and described.

I claim as my invention:

1. An electron emissive electrode for luminous tubes comprising a lead-in conductor 75 embedded in a sintered mass of nickel, barium oxide and strontium oxide.

2. An electron emissive electrode for luminous tubes comprising a lead-in conductor having one end thereof embedded in a sintered mass of nickel, barium oxide and strontium oxide.

3. An electron emissive electrode for luminous tubes comprising a refractory non-metallic sleeve, a lead-in conductor having an 85 end extending into the sleeve, and a sintered compact mass of nickel, barium oxide and strontium oxide in the sleeve, said mass being fused to the sleeve and lead-in conductor.

4. An electron emissive electrode for luminous tubes comprising a lead-in conductor and a sintered mass of one or more alkaline earths and nickel fused to said conductor.

5. An electron emissive electrode for luminous tubes comprising a homogeneous mass 95 of approximately the proportions by weight, nickel 50 percent, barium oxide 25 percent and strontium oxide 25 percent.

6. An electrode for luminous tubes utilizable either as a cathode or an anode, said electrode comprising a lead-in conductor, and a homogeneous mass of approximately the proportions by weight, nickel 50 percent, barium oxide 25 per cent and strontium oxide 25 percent, said mass being fused to an 105 end portion of the lead-in conductor that extends into the press end of the tubes.

7. The method of making electron emissive electrodes for luminous tubes that comprises filling a hollow refractory sleeve with 110 a mixture of nickel, barium carbonate and strontium carbonate, tamping said mixture and then heating the sleeve and mixture to form a sintered mass of nickel, barium oxide and strontium oxide.

8. The method of making electron emissive electrodes for luminous tubes that comprises inserting a lead-in conductor into a sleeve, filling a portion of said sleeve with a mixture of nickel, barium carbonate and strontium carbonate, compacting said mixture in the sleeve and about the lead-in conductor, and heating the mixture to form a sintered mass of nickel, barium oxide and strontium oxide.

9. An electron emissive electrode for luminous tubes comprising a lead-in conductor and a sintered mass of one or more alkaline earths and a non-oxidized metal of the ferrous group fused to said conductor.

10. An electron emissive electrode for luminous tubes comprising an elongated cylindrical member consisting of a homogeneous mass of one or more alkaline earths and nickel sintered together and having a lead-in conductor electrically connected to one end thereof and terminating within the sintered mass.

5 In testimony whereof, I have hereunto subscribed my name this 31st day of October,  
1928.

10 JOSEPH E. GROSS.

15

20

25

30

35

40

45

50

55

60

65